

Patented Feb. 23, 1926.

1,574,357

# UNITED STATES PATENT OFFICE.

MURRAY C. BEEBE AND ALEXANDER MURRAY, OF CINCINNATI, OHIO, ASSIGNORS TO THE WADSWORTH WATCH CASE COMPANY, OF DAYTON, KENTUCKY, A CORPORATION OF KENTUCKY.

## PHOTOGRAPHIC MEDIA AND PROCESS.

No Drawing.

Application filed August 31, 1922. Serial No. 585,517.

To all whom it may concern:

Be it known that we, MURRAY C. BEEBE (a) and ALEXANDER MURRAY (b), (a) is a citizen of the United States, (b) is a subject 5 of Great Britain, both residing at Cincinnati, in the county of Hamilton and State of Ohio, have invented certain new and useful Improvements in Photographic Media and Processes, of which the following is a 10 specification.

This invention relates to improved photographic media and processes.

The primary object is to provide an improved photographic medium which is capable of being used advantageously in the 15 industrial arts for varied purposes. The invention provides an improved light-sensitive, varnish-like medium adapted for various uses, a process of preparing such medium, and a photo-process employing the 20 improved photo-sensitive medium.

In accordance with the preferred practice 25 of the invention, a suitable oil is thickened to a state of incipient gelation and is incorporated in a varnish suitable for photographic uses, where further thickening, polymerizing, or hardening is selectively accomplished by the action of light projected 30 upon or transmitted to a coating of the material in accordance with an image, design, or character upon a transparency through which the light is transmitted.

Also, in accordance with the preferred 35 practice of the invention, use is made of accelerating agents in an improved manner. Preferably, these accelerating agents are used in a varnish which comprises a light-sensitive oil, and preferably such oil is preparatorily thickened to a state of incipient 40 gelation. However, in this aspect, the invention is broad, and the accelerating agents may be used in accordance with the invention in a medium comprising any suitable constituents which are adapted to be hardened, 45 set or rendered insoluble with respect to developing agents, selectively, under the action of light. It is preferred to employ as accelerating agents both a halogen-substituted hydrocarbon, such as iodoform, or 50 an equivalent compound, and a metallic halide, such as an iodide of lead, and, in addition, one may employ, if desired, small proportions of ingredients useful as driers, such as metal resinate, oxides, etc., com-

monly employed as paint or varnish driers. 55 If desired, moreover, such driers may be converted largely or wholly into metallic halides by introducing a halogen, for example, iodine, into the medium. The halogen compounds which are formed are dispersed throughout the medium in colloidal form, and, under the action of light, will liberate halogen which can thus serve as a catalytic agent in the transformation which occurs under the action of light. 60

The thickening of the oil, or oils, may be accomplished by heating, oxidation, destructive distillation, halogenation, hydrogenation, vulcanization, etc.

In place of incipiently gelled oils, one may 70 employ, with such special catalysts, other suitable bases such as resins, fats, waxes, bitumens, rubber, etc. Any suitable combination of materials may be effected.

Some of the bases are particularly adapted 75 to projection printing, and others are adapted to contact printing. The accelerating agents may be introduced into the medium in various ways, as will be understood more fully from the description hereinafter given.

When a coating comprising a base of the character herein described and a suitable accelerating agent is applied as a coating to a suitable surface and is subjected to the selective action of light in accordance with a projected or transmitted image, there occurs a selective hardening or setting of the coating, or a selective change in solubility. 85 those portions transformed under the action of light becoming, ordinarily, insoluble in developing agents. Thus, there is formed in the coating an image which will remain on the coated surface after the soluble portions have been removed in the developing 90 operation. Over printing may produce a reversal as to solubility or insolubility, as explained later.

Without intending to limit the invention, except as may be necessary in view of the 100 prior art, examples and steps are hereafter described which will enable the invention to be understood.

In the practice of the invention, one may 105 use as bases various substances, such as tung oil, perilla oil, soy bean oil, lard oil, cotton seed oil, fish oil, castor oil, linseed oil, menhaden oil, gutta percha, caoutchouc, fossil

and semi-fossil resins, fatty acids, waxes, bitumens, including so-called drying and non-drying oils, kerosene, synthetic resins, esters, etc., such as cellulose acetate.

- 5 It has been found that the various bases enumerated are naturally slightly sensitive to the action of light. In application, Serial No. 516,865, filed November 21, 1921, there is described a process employing preferably 10 a varnish which utilizes that property of Chinawood oil, combined with a suitable sensitizer or accelerator, whereby selective drying, or hardening, under the action of light occurs. In application, Serial No. 15 542,124, filed March 8, 1922, light-sensitive varnishes employing oils and method of preparing such varnishes are set forth; and the production of latent images in such varnishes on the principle of selective drying, hardening, or insolubilizing oleaginous media in accordance with a projected or transmitted light image is described. The present invention utilizes such oils in light-sensitive varnishes, and also comprises the 20 use of broadly equivalent bases, but the oils employed are preparatorily subjected to a thickening or polymerizing process which carries them to a state of incipient gelation near the critical point, leaving the 25 oils in such condition that they can be quickly transformed into such a state of insolubility as is desirable for the purposes of the invention.

It may be said, in general, that any non-aqueous colloid, which changes from sol to a gel condition in the light, or exhibits 30 selective solubility under the action of light, especially in the presence of a halogen, a metal salt, or other accelerator, or combination 35 of accelerators, may be used.

Continued research has shown that the precise chemical reactions cannot be fully specified, for the reason that the useful efficiency of such light-sensitive substances, 40 forming bases, depends, among other things, upon their varying physical properties, such as solubility, state of aggregation, dispersion, and internal structure.

Among many accelerators that may be 45 used, we have found that the following operate efficiently with the bases enumerated: metallic resinate, oleates, linoleate, tungates, etc., or any soluble salt particularly of lead, cobalt, manganese, copper, mercury, 50 silver, cadmium, bismuth, etc., alone or in combination with each other or with the halogens, iodine, chlorine, bromine, or compounds thereof, singly or in combination. We have also further found that phosphorus, 55 aluminum chloride and aluminum bromide act as accelerators, and in addition such catalysts as are recognized as suitable for halogenation.

In the main, it may be said that the bases mentioned are more or less light-sensitive.

For instance, cooked tung oil at the end of fifteen minutes' exposure indicates a reaction to light. The addition of iodine, alone, to cooked tung oil does not increase its sensitivity very greatly; the addition of lead 70 resinate, alone, which is itself sensitive to light action, increases the sensitivity of the cooked tung oil considerably; and the addition of both lead resinate and iodine to cooked tung oil increases the speed of printing very considerably. Such additions of lead resinate and iodine are desirable up to a certain point only. Beyond such point, which may be a saturation point, an increase 75 in these ingredients, and especially in iodine, 80 is not desirable. In general, the accelerators are to be used in relatively small proportions, as indicated by the examples hereinafter given. As has been indicated, light-sensitive oils, like tung oil, are made more sensitive 85 by the addition of lead resinate, manganese peroxide, lead peroxide, etc. Also, we have found that cobalt linoleate or lead oleate in benzol (benzene), with iodine, is sensitive to light action. Also, lead resinate 90 and iodine in a solution of gutta-percha and benzol produce a light-sensitive medium, which, under varying light action, becomes selectively insoluble in a manner similar to the other substances which have been mentioned. 95

In media which are slightly sensitive to light, a visible image may be produced. However, such image is not always easily developed by a solvent which will act efficiently in cases where accelerators are employed in the media. When, under such circumstances, the solvent does not entirely remove the base, such base will, due to the varying light action, have selective properties whereby it will variably absorb stains. The simplest form of developer which readily dissolves the unreacted part of the sensitive base is soap and water. 105

A reversed image, from the same subject 110 is produced by overprinting. With some mixtures, even better positives are secured than negatives. As an example, we have found by actual demonstration that a negative print is secured in fifteen seconds and 115 under the same conditions of light, etc., a positive is secured in an exposure of twenty seconds. In general terms, reversal is secured by approximately doubling the exposure. The sensitivity of cooked tung oil 120 alone is such as to give an impression in fifteen minutes, while with the addition of accelerators having catalyzing characteristics the exposure has been reduced to but two seconds under the same conditions. 125

While it has been known that some oils, such as tung oil, are somewhat sensitive to light, it may be stated that the raw oils do not become highly sensitive, even when accelerators are added. By thickening the oils 130

to a state of incipient gelation in accordance with the present invention, their light-sensitivity can be increased very greatly, and, in some cases, hundreds of times. Among the 5 special treatments which may be employed for preparing the oils, we may mention that when heat is applied to many oleaginous substances they gradually thicken or polymerize. By continuing the heating sufficiently long, a solid insoluble substance is 10 finally obtained. The heating is to be discontinued before that condition is reached. Of the numerous oils mentioned above, tung oil most rapidly reaches this condition. 15 Moreover, tung oil, when thus heated, reaches a rather sharply defined critical point, beyond which, if the heating is continued, the oil will quickly change to a complete gel. As the oil approaches the state of incipient gelation, the aggregates having molecular characteristics increase in size, thus decreasing their degree of dispersion. In ingredients of this kind, during the period of cooking, at the critical point of incipient gelling, 20 before the change to a full gel, they are in a condition of maximum sensitivity to light and are also in condition to be readily incorporated with suitable solvents and thinning agents to form a light-sensitive varnish. 25 In preparing a non-aqueous light-sensitive medium, it is preferable to start with tung oil, subject it to heat to the point of incipient gelling, and combine it with photographically cooperating diluents, accelerators, etc.

It should be stated that many organic materials have similar characteristics, and so may be used as bases. Among these may be mentioned gutta percha, fossil and semi-fossil resins, asphaltites, synthetic resins and esters such as cellulose acetate, vinyl acetate, etc., and waxes because they manifest sensitivity to light in an analogous manner. We have formed images by the use of these alternative materials which are similar in appearance and also show properties found in images produced on coatings composed of suitably treated oils, etc. In the other applications hereinbefore identified, iodine and the metallic compounds mentioned therein, are now more definitely referred to and we find that in addition bromine and chlorine or combinations of these are even more effective than one halogen alone. We also find that compounds of the halogens which liberate halogens under the action of light in the presence of the base have certain applications. Among such substances may be mentioned iodates, tetra iodo pyrrole, iodoform, bromoform, halogen sorption products of dye stuffs, etc.

We have found that the sensitivity of an oil is further increased by oxidation, so that, for example, by aerating or "blowing" tung oil, that is, heating the oil to about 85° C.

and passing air through it, and adding only traces of an accelerator the time for printing is only two minutes. Through the use of cooperating accelerators the time of printing is reduced to a few seconds.

We are not limited to the use of drying or semi-drying oils, as so-called non-drying oils may be thickened or polymerized to the point of incipient gelling by destructive distillation, halogenation, hydrogenation, vulcanization, or otherwise. For instance, castor oil is thickened by distilling off the lighter constituents until the residue begins to polymerize, at which time the addition of accelerators yields a light sensitive medium. Lard oil thickened by chlorination and heated to a highly viscous stage is light sensitive and may be accelerated in the same manner as the drying oils. Kerosene becomes available in our process by halogenation and dehalogenation which converts it into an unsaturated oil.

In the earlier applications referred to, the accelerating action of various pigments, especially of the oxides, was described. In some cases we have found that re-agents such as phosphorus, or others that are soluble in the medium but which precipitate as insoluble compounds under the influence of light, act as accelerators to completely gel the incipiently gelled medium, and thus give greater printing selectivity for contrast. In this connection, for example, we have found that lead iodide forms more rapidly in the light than in the dark.

In general, we have observed that the image grows from the supporting surface and that the nature of the surface has an important influence on the sensitivity and other properties of the print. For example, less exposure is required on a zinc than on a copper or brass support. Where it is desirable to modify the effect of the supporting surface a protective film of a dye, shellac, lacquer, glue, albumen, etc., may be used.

We have also found, as previously stated, that the speed of printing by our process is greatly accelerated by heat, which may be supplied in the form of a blast of hot air to the image during its exposure. It has also been found that minute quantities of halogen carriers, such as aluminum chloride, aluminum bromide, antimony chloride, also phosphorus, phosphorus oxychloride, etc., fluorescent dyes such as rhodamine, phenosafranine, eosine, etc., become cooperative accelerators to the main reactions.

The surface which is to receive an image is coated with the sensitive medium by flowing, brushing, spraying, whirling, etc. The surface may then be exposed for the requisite time and thereafter developed with a solvent that removes the unconverted portions of the coating. The remaining parts of the coating may serve to receive the action of

any suitable mordant or to confine the action of an etching agent to the areas laid bare. Our light-sensitive media are specially adapted, to the successful production 5 of photographic images, whether in continuous tone or otherwise. Attempts made heretofore to do this have not proved practical because of the slow reaction to light of the coating mediums used. The improved 10 varnish may be used very advantageously in the industrial arts. It may, for example, be used in the photographic processes set forth in the application of Murray C. Beebe, No. 542,124, mentioned above.

15 We do not limit ourselves to the employment of optical projection, as under certain conditions our sensitive coatings are sufficiently dry to admit of contact printing.

For contact printing, we have found advantages in using a solid colloid, such as lead oleate or bitumen or gutta percha in combination with a halogen or a halogen-forming substance, e. g. tetra-iodopyrrole or iodoform, the halogen liberated by light rendering the solid or "dry" film selectively soluble in suitable developers, such as fatty acids, concentrated or diluted.

As an instance of procedure with a base other than tung oil, we may state that a varnish composed of 100 gms. incipiently gelled linseed oil, 20 gms. cumar resin, 40 gms. kauri resin, 10 gms. lead tungate, 50 cc. solvent naphtha and 30 cc. benzol (benzene) may be used. 50 gms. of this varnish sensitized 30 with 20 cc. of a 5% solution of iodine in benzol and 5 cc. of a 5% solution of pyridine in benzol is sufficiently sensitized to produce a print under a two minute exposure.

By preparing a perilla oil varnish in substantially the same way and sensitized in the same way as above referred to, the time of printing under the same lighting conditions is reduced to about one sixth of the time mentioned for the linseed oil composition. Prints made in this manner are developable in a number of different ways, one 40 of which requires about one minute by means of a solution of 150 cc. butyl alcohol, 25 cc. benzine, 10 cc. terpineol. The prints, after 50 development, may be washed in alcohol and stained in any desired manner, such for instance, as by a solution of 150 cc. butyl alcohol, 150 cc. benzine, 25 cc. carbon tetrachloride, 30 gms. oil blue dye, and 20 gms. phenol, after which they are further washed 60 out with alcohol and dried. If desired the printed and developed images may be hardened by immersing them in a solution of aluminum chloride, iodine in potassium iodide solution, tannic acid, etc.

As a further exemplification, a tung oil varnish prepared and sensitized as follows, exposed by projection, and developed with soap and water, gives prints in a few seconds, under similar lighting conditions to

the linseed oil adaptation; such a varnish is composed of 32% tung oil, 3% lead resinate, 62.0% benzol and 3% iodine. The oil is treated by heating with the lead resinate for 30-60 minutes at 250° C.

In addition, a gutta percha adaptation 70 will give a print under lighting conditions similar to the previous exemplifications, by projection or contact, in about five minutes. A working relation of ingredients is exemplified in the following: gutta percha, 8.6%, carbon tetrachloride 55.2%, benzol 34.5%, iodine 0.85% and lead resinate 0.85%. Development may proceed with an application 75 of benzine.

The oils, fats, etc. ordinarily contain unsaturated fatty acids, or glycerides of fatty acids, which doubtless play an important part in the transformation which occurs in the medium under the selective action of 80 light.

From the description given, it will be understood that incipiently gelled oil and other bases mentioned are equivalents in the broad sense that they afford constituents in the 90 varnish which are of thick consistency, but which may be dissolved and carried as hydrophobic colloids in a suitable solvent and thinning medium, and are capable of being rapidly transformed selectively to an insoluble condition under the action of light. Also, that these substances afford constituents which are quickly converted to the insoluble state through the influence of halogen liberated under the action of light. The expression "gell-like body", as employed in appended claims, is intended to include incipiently gelled oils, as well as other bases, having the characteristics of gels, resins, etc., 95 mentioned above. As indicated, however, some of these bodies which are suitable bases may, in some state or condition, assume either a soft resinous form or a solid resinous form. They have, in general, a plastic or semi-plastic character before being dissolved 100 and thinned.

The expressions "oil red", "oil blue", "oil yellow", etc. are applied to dye stuffs which are insoluble in water, but soluble in oil. As non-aqueous colloids are used in the present process, it may be desirable to dye the film to enable the progress of development to be noted. Any oil dye, provided the medium in which it is dissolved does not also dissolve the printed image, may be used. 115 "Oil red" has been found to be a good dye to use for this purpose, because, while it is soluble in oil and not in water, it is, nevertheless, also soluble in alcohol. When a varnish coating is printed and then dipped in an alcoholic solution of oil red dye, the alcohol does not destroy the image, but the dye produces a deep color in the image which is of assistance in watching the development.

120 It may be added that a number of the 130

- halogen-liberating compounds heretofore mentioned as being suitable for use as sensitizers, such as iodoform, bromoform, and tetra-iodopyrrole, may be classified as organo halogen compounds, which, in this process are halogen-liberating compounds. Such compounds are especially useful as sensitizers in connection with non-aqueous, or hydrophobic, colloids which are capable of being transformed, or hardened, under the action of light.
- The foregoing detailed description has been given for clearness of understanding only, and no unnecessary limitations should be understood therefrom, but the appended claims should be construed as broadly as permissible, in view of the prior art.
- What we regard as new, and desire to secure by Letters Patent, is:
20. 1. A photographic medium comprising a suitable base, which base comprises a hydrophobic gell-like body sensitive to the action of light, and a catalytic accelerator incorporated with said base.
  25. 2. A photographic medium comprising a suitable base which comprises a hydrophobic gell-like body sensitive to the action of light, and an accelerator which serves as a catalyst in the transformation of said body under the action of light.
  30. 3. A photographic medium comprising an incipiently gelled oleaginous base, and an accelerator adapted to expedite the transformation of said base under the action of light.
  35. 4. A photographic medium comprising an incipiently gelled oleaginous base which comprises a fatty acid compound, and an accelerator having, under the action of light, a catalytic action facilitating the transformation of said base.
  40. 5. A photographic medium comprising a light-sensitive varnish which comprises a light-sensitive incipiently gelled oil.
  45. 6. A photographic medium comprising an incipiently gelled oil adapted to be transformed under the action of light, and an accelerator serving to expedite such transformation.
  50. 7. A photographic medium comprising an incipiently gelled oil adapted to be transformed under the action of light, and an accelerator acting as a catalyst under the influence of light.
  55. 8. A photographic medium comprising a base which comprises a non-aqueous gell-like body capable of being transformed under the action of light, and an accelerator comprising a halogen-liberating compound.
  60. 9. A photographic medium comprising a varnish which comprises a non-aqueous gell-like body capable of being transformed under the action of light, and a halogen-liberating agent.
  65. 10. A photographic medium comprising an incipiently gelled body comprising fatty acid compounds, a natural resin-like compound, and an accelerating agent adapted to accelerate the selective action of light upon said medium when the medium is subjected to photographic action.
  70. 11. A photographic medium comprising an incipiently gelled oil, a natural resin-like compound, an accelerating agent adapted to accelerate the selective action of light upon said medium when the medium is subjected to photographic action, and a diluent.
  75. 12. A photographic medium comprising a base which comprises: a gell-like body sensitive to the action of light, and accelerating means comprising a halogen-substituted hydrocarbon and a metallic halide.
  80. 13. A photographic medium comprising an incipiently gelled oil, a natural resinous compound, and accelerating means comprising a halogen-substituted hydrocarbon and a metallic halide.
  85. 14. A photographic medium comprising an incipiently gelled oil, a natural resinous compound, an accelerating agent comprising a halogen-substituted hydrocarbon and a metallic halide, and a diluent.
  90. 15. A photographic medium comprising incipiently gelled tung oil, and an accelerating agent adapted to accelerate the selective action of light upon said medium when the medium is subjected to photographic action.
  95. 16. A photographic medium comprising incipiently gelled tung oil, a natural resinous compound, and an accelerating agent adapted to accelerate the selective action of light upon said medium when the medium is subjected to photographic action.
  100. 17. A photographic medium comprising incipiently gelled tung oil and accelerating means comprising a halogen-liberating compound.
  105. 18. A photographic medium comprising incipiently gelled tung oil and halogen-liberating means comprising a halogen-substituted hydrocarbon and a metallic halide.
  110. 19. A photographic medium comprising a suitable base which comprises: a gell-like body sensitive to the action of light, and accelerating means comprising iodoform.
  115. 20. A photographic medium comprising a suitable base which comprises: a hydrophobic gell-like body sensitive to the action of light, and accelerating means comprising iodoform and an iodide.
  120. 21. A photographic medium comprising a suitable base which comprises: constituents adapted to be transformed under the action of light, and accelerating means comprising a halogen-substituted hydrocarbon and a metallic halide.
  125. 22. A photographic medium comprising a suitable base of gell-like character and sensitive to the action of light, and accelerating

means comprising halogen-substituted hydrocarbon and a metallic halide.

23. A photographic medium comprising a suitable base of gell-like character and sensitive to the action of light, and accelerating means comprising a metallic halide and an additional halogen-liberating agent.

24. A photographic medium consisting of a varnish comprising a suitable base of gell-like character and sensitive to the action of light, an accelerator comprising a metallic halide and an additional halogen-liberating compound, and a diluent.

25. A photographic medium comprising a suitable base which is light sensitive, and accelerating means which comprises a plurality of different halogen-liberating compounds.

26. A photographic medium comprising a non-aqueous, light-sensitive colloid, a medium in which said colloid is carried, and accelerating means comprising a metallic halide and another halogen-liberating compound.

27. The process of preparing a light-sensitive medium which comprises: incorporating with a base which comprises a gell-like non-aqueous colloid which is sensitive to the action of light an accelerating agent adapted to expedite the transformation of said colloid under the action of light.

28. The process of preparing a light-sensitive medium, which comprises: incorporating with a base which comprises a gell-like non-aqueous colloid which is sensitive to the action of light, accelerating means comprising a metallic halide and another halogen-liberating compound.

29. The process of preparing a photographic medium which comprises: incorporating with a non-aqueous gell-like colloid an accelerator comprising a metallic halide and another halogen-liberating compound; and incorporating also therewith a diluent.

30. The process of preparing a photographic medium which comprises: producing an incipiently gelled oil and incorporating therewith an accelerating agent.

31. The process of preparing a photographic medium which comprises: producing an incipiently gelled oil and incorporating therewith accelerating means comprising a metallic halide and another halogen-liberating compound.

32. The process of preparing a photographic medium which comprises: producing an incipiently gelled oil and incorporating therewith accelerating means comprising a metallic halide and a halogen-substituted hydrocarbon.

33. The process of forming a light-sensitive medium which comprises: forming an incipiently gelled oil, incorporating therewith accelerating means comprising a metallic halide and another halogen-liberating

compound, and incorporating also therewith a diluent.

34. The process of forming a light-sensitive medium which comprises: producing an incipiently gelled oil and incorporating therewith a natural resinous compound and an accelerator.

35. The process of forming a light-sensitive medium which comprises: producing an incipiently gelled oil and incorporating therewith a natural resinous compound and an accelerator comprising a metallic halide and another halogen-liberating compound.

36. The process of forming a light-sensitive medium which comprises: reducing an oil to an incipiently gelled condition and incorporating therewith a halogen-liberating agent.

37. The process of producing a light-sensitive medium which comprises: reducing tung oil to an incipiently gelled condition, incorporating therewith an accelerator which comprises a halogen-liberating agent, and combining the said ingredients with a thinning agent.

38. The process of producing a resistant image, design, or character on a surface which comprises: applying to said surface a coating comprising a gell-like base which is capable of being transformed into a hardened state, a solvent and thinning medium carrying said base, and an accelerator; acting upon said coating selectively with light in accordance with an image, design, or character to effect the desired transformation; and subjecting the coating to a developing operation.

39. The process of producing a resistant image, design, or character on a surface which comprises: applying to said surface a coating comprising a gell-like base which is capable of being transformed into a hardened state, a solvent and thinning medium carrying said base, and an accelerator comprising a halogen-liberating compound; acting upon said coating selectively with light in accordance with an image, design, or character to effect the desired transformation; and subjecting the coating to a developing operation.

40. The process of producing a resistant image, design, or character on a surface which comprises: applying to said surface a coating comprising a gell-like base which is capable of being transformed into a hardened state, a solvent and thinning medium carrying said base, and an accelerator comprising a metallic halide and another halogen-liberating compound; acting upon said coating selectively with light in accordance with an image, design, or character to effect the desired transformation; and subjecting the coating to a developing operation.

41. The process of producing a resistant

- image, design, or character on a surface which comprises: applying to said surface a coating which comprises an incipiently gelled oil, a suitable solvent and thinning medium, and a halogen-liberating compound; acting upon said coating selectively with light transmitted in accordance with an image, design, or character; and developing the print.
- 10 42. A photographic medium comprising hydrophobic colloids adapted to be transformed under the action of light, and accelerating means comprising an organo-halogen compound adapted to liberate halogen under the action of light.
- 15 43. A photographic medium comprising hydrophobic colloids adapted to be transformed under the action of light, and accelerating means comprising a halogen-substituted hydrocarbon.
- 20 44. A photographic medium comprising hydrophobic colloids adapted to be transformed under the action of light, and accelerating means comprising iodoform.
- 25 45. A photographic medium comprising a solution of a hydrophobic colloid adapted to be transformed under the action of light, and accelerating means comprising an organo-halogen-liberating compound.
- 30 46. The process of preparing a light-sensitive medium which comprises: incorporating with a base which comprises a non-aqueous colloid adapted to be transformed under the action of light an accelerating agent comprising an organo-halogen compound adapted to liberate halogen under the action of light.
- 35 47. A photographic process which comprises: applying to a surface a coating comprising hydrophobic colloids capable of being transformed into a hardened state under the action of light and having incorporated therein an organo-halogen-liberating compound; and subjecting said coating to the selective action of light in accordance with an image, design or character.
48. A photographic process which comprises: applying to a surface a coating comprising hydrophobic colloids capable of being transformed into a hardened state under the action of light and having incorporated therein an organo-halogen-liberating compound; subjecting said coating to the selective action of light in accordance with an image, design or character; and subjecting the coating to a developing operation.
- 50 49. A photographic process which comprises: applying to a surface a coating composed of a solution comprising hydrophobic colloids capable of being transformed into a hardened state under the action of light and having incorporated therein a halogen-substituted hydrocarbon; and subjecting said coating to the selective action of light 60 in accordance with an image, design or character to effect the desired transformation.
- 55 50. A photographic process which comprises: applying to a surface a coating composed of a solution comprising hydrophobic colloids capable of being transformed into a hardened state under the action of light and having incorporated therein iodoform; and subjecting said coating to the selective action of light in accordance with an image, 70 design or character to effect the desired transformation.
- 58 51. A photographic process which comprises: applying to a surface a coating composed of a solution comprising hydrophobic colloids capable of being transformed into a hardened state under the action of light and having incorporated therein iodoform; subjecting said coating to the selective action of light in accordance with an image, 80 design or character to effect the desired transformation; and subjecting the coating to a developing operation.
- In testimony whereof we affix our signatures.
- MURRAY C. BEEBE.  
ALEXANDER MURRAY.